

# United States Patent Office

2,916,401

Patented Dec. 8, 1959

1

2,916,401

## CHEMICAL REDUCTION NICKEL PLATING BATH

Lawrence V. Puls, Ferndale, and William R. Vincent, Birmingham, Mich., assignors to General Motors Corporation, Detroit, Mich., a corporation of Delaware

No Drawing. Application February 10, 1958  
Serial No. 714,077

13 Claims. (Cl. 117—130)

This invention relates to an improved bath and process for nickel plating by chemical reduction.

It is well known that various metals may be nickel plated by chemical reduction in an aqueous bath containing nickel ion and hypophosphite ion, the plating reaction being:



This reaction whereby the plating occurs is catalytic and autocatalytic, its initiation usually being accomplished by way of the catalytic effect of the article being plated and its continuance being catalyzed by the nickel which is deposited. Various metals may be plated by the process, for example, copper, gold, aluminum, iron, nickel, silver, cobalt, palladium, platinum. Magnesium and thorium also display the catalytic effect and theoretically, therefore, may be plated by the process; however, the plating of these metals has presented a serious problem in that when they are immersed in baths such as have heretofore been used, they are chemically attacked by the solution with the result that a satisfactory plate is not obtained.

It is an object of the present invention to provide an improved electroless nickel plating bath and process which is particularly useful for nickel plating magnesium and also thorium. Another object of the invention is the provision of an electroless nickel plating bath and process which provides an improved nickel deposition and which has improved stability even in the presence of magnesium and thorium. While the bath and process have particular utility and advantages in the plating of magnesium and thorium, other metals such as those mentioned above may also be plated, the improved stability and the high plating rate of the bath and process being highly advantageous irrespective of the precise metal being plated. Other objects and advantages of the invention will appear more fully from the following description of various embodiments thereof.

In accordance with the invention the aqueous nickel plating bath is formulated to contain the following ingredients in the concentration indicated:

|                                                  |                                                                                        |
|--------------------------------------------------|----------------------------------------------------------------------------------------|
| Nickel ion.....                                  | From .005 to .20 mole per liter.                                                       |
| Hypophosphite ion.....                           | From .01 to .40 mole per liter.                                                        |
| Fluoride ion.....                                | From .20 to 1.0 mole per liter.                                                        |
| Alkyl or alkanol amine.....                      | Sufficient to provide an N to Ni <sup>++</sup> ratio of from 1:1 to 10:1.              |
| Carboxylic acid or salt thereof as a buffer..... | Sufficient to produce a carboxyl group-to-hypophosphite ion ratio of from 1:1 to 10:1. |

Initial pH..... 7 to 11.

The nickel ion may be added as nickel acetate or nickel sulphate and the hydrophosphite as sodium hypophosphite, potassium hypophosphite or hypophosphorous acid. For the source of the fluoride ion, it is preferable to use ammonium bifluoride, though sodium fluoride, potassium fluoride or hydrofluoric acid may be used if desired. The carboxylic acid radical used as a buffer may, for example, be acetate, propionate, succinate, lactate, glycolate or citrate, added either as the acid or as a sodium or similar soluble salt thereof. As indicated by these ex-

2

amples, the carboxylic acid used as the buffer may be a polycarboxylic acid or an hydroxy carboxylic acid. Since a polycarboxylic acid furnishes more carboxyl groups per mole than does a monocarboxylic acid, their use is generally desirable. We prefer to use citric acid as the buffer.

The amine must be sufficiently soluble in the bath to provide the desired concentration, and must also have a sufficiently high boiling point so that it is not lost due to evaporation at the desired bath temperature which should be in the range of 130° F. to 210° F., preferably above 160° F. Amines which are satisfactory are any of the primary, secondary or tertiary ethyl amines or propyl amines, ethylene or propylene diamine, ethanol amine, di or tri ethanol amine, methanol amine, di or tri methanol amine, propanol amine, or di or tri propanol amine.

The initial pH of the bath, which is on the alkaline side, may be adjusted by addition of the amine ingredient or by the addition of sodium or potassium hydroxide.

For optimum results, however, it is preferred that the N to Ni<sup>++</sup> ratio be on the order of 5:1 and thus it is desirable to add just sufficient amine to provide this preferred ratio and then adjust the initial pH by the addition of potassium hydroxide or sodium hydroxide.

25 The following specific examples will serve to illustrate, Example I being the preferred bath by way of its precise ingredients and also by way of the amounts thereof which are used:

### Example I

|                                                                        |                       |     |
|------------------------------------------------------------------------|-----------------------|-----|
| 30 Nickel sulfate .....                                                | grams per liter ..... | 5.5 |
| Sodium hypophosphite .....                                             | do .....              | 8.3 |
| Citric acid .....                                                      | do .....              | 10  |
| Triethanolamine N(C <sub>2</sub> H <sub>5</sub> OH) <sub>3</sub> ..... | ml. per liter .....   | 20  |
| Ammonium bifluoride (NH <sub>4</sub> F·HF) .....                       | grams per liter ..... | 10  |
| pH (adjusted by addition of NaOH) .....                                | .....                 | 8.0 |
| Temperature .....                                                      | ° F .....             | 205 |

### Example II

|                                        |                       |            |
|----------------------------------------|-----------------------|------------|
| 40 Nickel sulfate .....                | grams per liter ..... | 5          |
| Sodium hypophosphite .....             | do .....              | 8.3        |
| Acetic acid .....                      | do .....              | 10         |
| Triethanolamine .....                  | ml. per liter .....   | Approx. 60 |
| Ammonium bifluoride .....              | grams per liter ..... | 10         |
| pH (adjusted by the amine added) ..... | .....                 | 8.0        |
| Temperature .....                      | ° F .....             | 190        |

### Example III

|                                                                       |                       |         |
|-----------------------------------------------------------------------|-----------------------|---------|
| 50 Nickel sulfate .....                                               | grams per liter ..... | 5.5     |
| Sodium hypophosphite .....                                            | do .....              | 8.3     |
| Citric acid .....                                                     | do .....              | 9       |
| Potassium fluoride .....                                              | do .....              | 11.8    |
| Ethanolamine NH <sub>2</sub> (C <sub>2</sub> H <sub>5</sub> OH) ..... | ml. per liter .....   | 9       |
| pH (adjusted by addition of KOH) .....                                | .....                 | 8.0     |
| Temperature .....                                                     | ° F .....             | 185-190 |

### Example IV

|                              |                       |         |
|------------------------------|-----------------------|---------|
| 60 Nickel sulfate .....      | grams per liter ..... | 11      |
| Sodium hypophosphite .....   | do .....              | 16.6    |
| Citric acid .....            | do .....              | 17      |
| Potassium fluoride .....     | do .....              | 21.7    |
| Triethanolamine .....        | mls. per liter .....  | 40      |
| pH (adjusted with KOH) ..... | .....                 | 8.1     |
| Temperature .....            | ° F .....             | 185-190 |

### Example V

|                                                                    |                       |            |
|--------------------------------------------------------------------|-----------------------|------------|
| 65 Nickel sulfate .....                                            | grams per liter ..... | 5          |
| Sodium hypophosphite .....                                         | do .....              | 8.3        |
| Citric acid .....                                                  | do .....              | 8          |
| Ammonium bifluoride .....                                          | do .....              | 8          |
| Triethylamine N(C <sub>2</sub> H <sub>5</sub> ) <sub>3</sub> ..... | mls. per liter .....  | Approx. 80 |
| pH (adjusted by the amine added) .....                             | .....                 | 10.85      |
| Temperature .....                                                  | ° F .....             | 210        |

**3**  
**Example VI**

|                         |                 |      |
|-------------------------|-----------------|------|
| Nickel sulfate          | grams per liter | 17.6 |
| Sodium hypophosphite    | do              | 26.6 |
| Ammonium bifluoride     | do              | 27.8 |
| Citric acid             | do              | 180  |
| Ethanolamine            | moles per liter | 50   |
| pH (adjusted with NaOH) |                 | 8.0  |
| Temperature             | ° F.            | 135  |

To practice the process of the invention, the magnesium, thorium or other metal article to be plated is first thoroughly cleaned by conventional degreasing and chemical cleaning procedures and is then immersed into the bath until the desired plating thickness is obtained. The precise plating rate attained is dependent upon the concentrations of the bath ingredients and also upon bath temperature. In general, the higher the nickel ion concentration and the higher the temperature, the faster the plating rate; however, with increased nickel concentration and with increased temperature the greater is the possibility of bath instability. The preferred bath as set forth in Example I provides an initial plating rate of about .0015 inch per hour which is excellent; at the same time, this bath is very stable and can therefore be operated on a production basis without the hazard of precipitation occurring.

After the bath has been operated for a time it may, if desired, be replenished by the addition of nickel ion, hypophosphite ion and potassium or sodium hydroxide. For example, a bath as specified in Example V above was operated until there was substantial depletion of the nickel ion (at which point the pH of the bath was 6.4) and then replenished by the addition of 9 grams nickel sulfate, 9 grams sodium hypophosphite and sufficient sodium hydroxide to raise the pH to 10.9. The replenished bath was then used again for further plating until the nickel was once more depleted. Also, replenishment may, if desired, be on a continuous basis so as to keep the bath in continuous operation for an extended period.

It is to be understood that while the invention has been described chiefly by reference to particular embodiments thereof, it is not so limited since various changes and modifications may be made, all within the full and intended scope of the claims which follow.

We claim:

1. A chemical reduction type nickel plating bath comprising an aqueous solution having an initial pH of between 7 and 11 and containing the following in the concentrations indicated:

|                        |                                                                           |
|------------------------|---------------------------------------------------------------------------|
| Nickel ion             | From .005 to .20 mole per liter.                                          |
| Hypophosphite ion      | From .01 to .40 mole per liter.                                           |
| Fluoride ion           | From .20 to 1.0 mole per liter.                                           |
| Alkyl or alkanol amine | Sufficient to provide an N to Ni <sup>++</sup> ratio of from 1:1 to 10:1. |

Carboxylic acid or salt thereof as a buffer.

2. A chemical reduction type nickel plating bath comprising an aqueous solution having an initial pH of between 7 and 11 and containing from .005 to .20 mole per liter nickel ion, from .01 to .40 mole per liter hypophosphite ion, from .20 to 1.0 mole per liter fluoride ion, sufficient amine to provide an N to Ni<sup>++</sup> ratio of from 1:1 to 10:1 and sufficient carboxylic acid buffer to produce a carboxyl group-to-hypophosphite ion ratio of from 1:1 to 10:1 and sufficient carboxylic acid buffer to produce a carboxyl group-to-hypophosphite ion ratio of from 1:1 to 10:1.

3. A chemical reduction type nickel plating bath comprising an aqueous solution having an initial pH of between 7 and 11 and containing from .005 to .20 mole per liter nickel ion, from .01 to .40 mole per liter hypophosphite ion, from .20 to 1.0 mole per liter fluoride ion, sufficient amine to provide an N to Ni<sup>++</sup> ratio of from 1:1 to 10:1 and sufficient carboxylic acid buffer to produce a carboxyl group-to-hypophosphite ion ratio of from 1:1 to 10:1, said amine being selected from the group consisting of the methyl, ethyl and propyl amines, the methanol, ethanol and propanol amines and the ethylene and propylene diamines.

4. A process for depositing nickel by chemical reduction comprising immersing the article to be plated in a bath maintained at a temperature of between 130° and 210° F., having an initial pH of between 7 and 11 and containing the following in the concentrations indicated:

|                                              |                                                                                        |
|----------------------------------------------|----------------------------------------------------------------------------------------|
| Nickel ion                                   | From .005 to .20 mole per liter.                                                       |
| Hypophosphite ion                            | From .01 to .40 mole per liter.                                                        |
| Fluoride ion                                 | From .20 to 1.0 mole per liter.                                                        |
| Alkyl or alkanol amine                       | Sufficient to provide an N to Ni <sup>++</sup> ratio of about 5:1.                     |
| Carboxylic acid or salt thereof as a buffer. | Sufficient to produce a carboxyl group-to-hypophosphite ion ratio of from 1:1 to 10:1. |

5. A chemical reduction type nickel plating bath comprising an aqueous solution having an initial pH of between 7 and 11 and containing the following in the concentrations indicated:

|                      |                 |     |
|----------------------|-----------------|-----|
| Nickel sulfate       | grams per liter | 5.5 |
| Sodium hypophosphite | do              | 8.3 |
| Citric acid          | do              | 10  |
| Triethanolamine      | ml. per liter   | 20  |
| Ammonium bifluoride  | grams per liter | 10  |

6. A process for depositing nickel by chemical reduction comprising immersing the article to be plated in a bath maintained at a temperature of between 130° and 210° F., having an initial pH of between 7 and 11 and containing the following in the concentrations indicated:

|                                              |                                                                                        |
|----------------------------------------------|----------------------------------------------------------------------------------------|
| Nickel ion                                   | From .005 to .20 mole per liter.                                                       |
| Hypophosphite ion                            | From .01 to .40 mole per liter.                                                        |
| Fluoride ion                                 | From .20 to 1.0 mole per liter.                                                        |
| Alkyl or alkanol amine                       | Sufficient to provide an N to Ni <sup>++</sup> ratio of from 1:1 to 10:1.              |
| Carboxylic acid or salt thereof as a buffer. | Sufficient to produce a carboxyl group-to-hypophosphite ion ratio of from 1:1 to 10:1. |

7. A process for depositing nickel by chemical reduction comprising immersing the article to be plated in a bath maintained at a temperature of between 130° and 210° F., having an initial pH of between 7 and 11 and containing the following in the concentrations indicated:

|                                              |                                                                                        |
|----------------------------------------------|----------------------------------------------------------------------------------------|
| Nickel ion                                   | From .005 to .20 mole per liter.                                                       |
| Hypophosphite ion                            | From .01 to .40 mole per liter.                                                        |
| Fluoride ion                                 | From .20 to 1.0 mole per liter.                                                        |
| Alkyl or alkanol amine                       | Sufficient to provide an N to Ni <sup>++</sup> ratio of from 1:1 to 10:1.              |
| Carboxylic acid or salt thereof as a buffer. | Sufficient to produce a carboxyl group-to-hypophosphite ion ratio of from 1:1 to 10:1. |

8. A process for nickel plating by chemical reduction an article made of a metal selected from the group consisting of magnesium and thorium, said process comprising immersing said article in a solution having an initial pH of between 7 and 11 and containing the following in the concentrations indicated:

|                                              |                                                                                        |
|----------------------------------------------|----------------------------------------------------------------------------------------|
| Nickel ion                                   | From .005 to .20 mole per liter.                                                       |
| Hypophosphite ion                            | From .01 to .40 mole per liter.                                                        |
| Fluoride ion                                 | From .20 to 1.0 mole per liter.                                                        |
| Alkyl or alkanol amine                       | Sufficient to provide an N to Ni <sup>++</sup> ratio of from 1:1 to 10:1.              |
| Carboxylic acid or salt thereof as a buffer. | Sufficient to produce a carboxyl group-to-hypophosphite ion ratio of from 1:1 to 10:1. |

9. A process for nickel plating by chemical reduction an article made of a metal selected from the group consisting of magnesium and thorium, said process comprising immersing said article in a solution having an initial pH of between 7 and 11 and containing from .005 to .20 mole per liter nickel ion, from .01 to .40 mole per liter hypophosphite ion, from .20 to 1.0 mole per liter fluoride ion, sufficient amine to provide an N to Ni<sup>++</sup> ratio of from 1:1 to 10:1 and sufficient carboxylic acid buffer to produce a carboxyl group-to-hypophosphite ion ratio of from 1:1 to 10:1, said amine being selected from the group consisting of the methyl, ethyl and propyl amines, the methanol, ethanol and propanol amines and the ethylene and propylene diamines.

the methanol, ethanol and propanol amines and the ethylene and propylene diamines.

10. A process for nickel plating by chemical reduction an article made of a metal selected from the group consisting of magnesium and thorium, said process comprising immersing said article in a solution having an initial pH of between 7 and 11 and containing from .005 to .20 mole per liter nickel ion, from .01 to .40 mole per liter hypophosphite ion, from .2 to 1.0 mole per liter fluoride ion, sufficient amine to provide an N to Ni<sup>++</sup> ratio of from 1:1 to 10:1 and sufficient carboxylic acid buffer to produce a carboxyl group-to-hypophosphite ion ratio of from 1:1 to 10:1, said amine being selected from the group consisting of the methyl, ethyl and propyl amines, the methanol, ethanol and propanol amines and the ethylene and propylene diamines, and said buffer being selected from the group consisting of acetic acid, propionic acid, succinic acid, lactic acid, glycolic acid, citric acid and the soluble salts thereof.

11. A process for nickel plating by chemical reduction an article made of a metal selected from the group consisting of magnesium and thorium, said process comprising immersing said article in a solution having an initial pH of between 7 and 11 and containing nickel sulfate sufficient to produce from .005 to .20 mole per liter nickel ion, sodium hypophosphite sufficient to produce from .01 to .40 mole per liter hypophosphite ion, ammonium bifluoride sufficient to produce from .2 to 1.0 mole per liter fluoride ion, triethanolamine sufficient to provide an N to Ni<sup>++</sup> ratio of from 1:1 to 10:1 and citric acid sufficient to produce a carboxyl group-to-hypophosphite ion ratio of from 1:1 to 10:1.

12. A process for nickel plating by chemical reduction an article made of a metal selected from the group consisting of magnesium and thorium, said process comprising immersing said article in a solution having an initial pH of between 7 and 11 and containing the following in the concentrations indicated:

Nickel ion ..... From .005 to .20 mole per liter.  
Hypophosphite ion ..... From .01 to .40 mole per liter.  
Fluoride ion ..... From .2 to 1.0 mole per liter.  
Alkyl or alkanol amine ..... Sufficient to provide an N to Ni<sup>++</sup> ratio of about 5:1.  
10 Carboxylic acid or salt thereof as a buffer. Sufficient to produce a carboxyl group-to-hypophosphite ion ratio of from 1:1 to 10:1.

13. A process for nickel plating by chemical reduction an article made of a metal selected from the group consisting of magnesium and thorium, said process comprising immersing said article in a solution having an initial pH of about 8 and containing the following in the concentrations indicated:

Nickel sulfate ..... grams per liter 5.5  
Sodium hypophosphite ..... do 8.3  
Citric acid ..... do 10  
Triethanolamine ..... ml. per liter 20  
Ammonium bifluoride ..... grams per liter 10

#### References Cited in the file of this patent

#### UNITED STATES PATENTS

|           |                |               |
|-----------|----------------|---------------|
| 2,694,017 | Reschan et al. | Nov. 9, 1954  |
| 2,694,019 | Gutzeit        | Nov. 9, 1954  |
| 2,772,183 | Talmey et al.  | Nov. 27, 1956 |